

## UNITED STATES PATENT OFFICE

GEORGE A. RICHTER AND CHESTER H. GOLDSMITH, OF BERLIN, NEW HAMPSHIRE, AS  
SIGNORS TO BROWN COMPANY, OF BERLIN, NEW HAMPSHIRE, A CORPORATION OF  
MAINE

## FINISHING OF VISCOSE-RAYON

No Drawing.

Application filed November 14, 1929. Serial No. 407,271.

This invention relates to the finishing of rayon, being more particularly concerned with the finishing of crude rayon produced by the so-called viscose-rayon process.

- 5 In the manufacture of viscose-rayon, the practice is to "spin" the viscose syrup through spinnerets into an acid salt bath which serves to set the syrup as filaments, which issue continuously from the bath as yarn. The crude 10 rayon yarn thus produced is usually accumulated in spool, cake, or skein form, and then is subjected to various chemical treatments designed to purify it and to improve luster, whiteness, softness, and other silk-like qualities. The crude yarn may vary in color from 15 amber to light tan, depending upon the process of manufacture and the purity of the cellulose pulp used as a raw material in the production of the viscose syrup. It is contaminated by the sulphur precipitated when the viscose is set in the acid bath, this impurity impairing its luster. The usual finishing of 20 viscose-rayon comprises desulphurizing and bleaching steps, desulphurization having 25 heretofore been effected before bleaching in order to ensure the removal of coloring substance generated during desulphurization, as well as those present in the original crude 30 yarn.
- 30 We have found that it is distinctly advantageous to effect the bleaching of the crude yarn before it is subjected to desulphurization, as the nascent yarn is evidently far more 35 resistant to the deteriorating action of the usual oxidizing bleaching agents, such as chlorine water, or calcium or sodium hypochlorite solutions. Experiments have demonstrated that, whereas the yarn undergoes marked loss in strength and is quite sensitive 40 to oxidation after treatment with solutions of desulphurizing agents such as sodium sulphide, it undergoes little, if any, loss in strength or oxidation if whitened with oxidizing bleaching agents prior to desulphurization. In order to avoid reaction between the 45 residual bleaching agent carried by the yarn after bleaching and desulphurizing agents such as sodium sulphide employed in the subsequent step of desulphurization, the bleached 50 yarn is preferably treated with a solution of a reducing agent capable of converting such residual bleach into inactive products. While it is possible to employ solutions of various water-soluble reducing agents for this purpose, we prefer to use water-soluble aldehydes, such as formaldehyde, sodium sulphite, or other water-soluble agents which do not react with and precipitate sulphur from the sulphide class of desulphurizing agents, such as sodium sulphide, ammonium sulphide, or the like. The use of such reducing agents makes possible dispensing with a step of washing after treatment with reducing agents, and at the same time permits using sulphide desulphurizing agents, which are advantageous in that they effect a more rapid and complete desulphurization than other classes of desulphurizing agents. After desulphurization has been effected, the yarn may be washed free of desulphurizing agent and reaction products, whereupon it is preferably superbleached with agents such as permanganate, sodium peroxide, or peroxide solutions which do not materially adversely affect the strength or other qualities of the yarn in concentrations and under such conditions as are necessary for merely a superbleaching operation. Such superbleaching agents may be more expensive than the bleaching agent used for bleaching the crude yarn, but it is necessary to employ only comparatively dilute solutions of such agents, as the yarn is already white, and when treated with these dilute solutions acquires brilliant whiteness. When permanganate solutions are employed for superbleaching, it is preferable that they be neutral or slightly acid, as alkaline permanganate solutions have been found to lower the strength of the yarn. After permanganate superbleaching, the yarn may be treated with a suitable reducing agent, such as a sulphurous acid solution, to reduce residual permanganate to colorless manganous salts, whereupon the yarn may be washed in a soap solution, which enhances softness and serves to deposit a soap film which acts as a lubricant during subsequent weaving or knitting operations.
- The process of the present invention may be applied to rayon after it has been accumu-

lated, for instance on spools or in centrifuge baskets, or has been reeled into skeins. It may, however, be practiced with especial advantage upon rayon coming from the setting bath before it is accumulated in accordance with the disclosure of application Serial No. 356,426, filed April 19, 1929, by George A. Richter. In actual practice, where multiple spinning machines are employed, the yarns 10 coming from one or a series of acid setting baths may be passed through a series of treating baths such as hereinafter described, before being accumulated. Assuming that the viscose syrup has been spun into the usual 15 acid setting bath, for instance a solution of sulphuric acid and sodium sulphate, the crude yarn issuing from the setting bath is preferably first washed free of acid solution carried thereby. This may be accomplished by passing 20 the yarn through a bath of water, for instance at 80° C., which not only serves to wash water-soluble constituents, including acid, from the yarn, but to convert any residual xanthate into regenerated cellulose. 25 The yarn may then be passed through a bath of suitable oxidizing bleach solution, for instance chlorine water or calcium or sodium hypochlorite bleach solution, containing 1% available chlorine and at 20° to 25° C. When 30 hypochlorite bleach is employed, it is preferable to maintain the bleach solution in slightly alkaline condition, as under such condition it is possible to preserve maximum strength of yarn. The bleach solution need contain only 35 about .04% caustic soda for this purpose. The bleached yarn is then passed through a bath of suitable reducing solution, for instance a 1% solution of formaldehyde at 20° to 25° C. Preferably, the formaldehyde 40 solution is also alkaline and contains an alkali such as caustic soda to the extent of about 1%, as the alkali accelerates the reaction between the formaldehyde and residual bleach carried by the yarn into the reducing 45 solution and further serves to prevent decomposition of the formaldehyde. The yarn is then passed through a bath of suitable desulphurizing solution, preferably containing a sulphide desulphurizing agent such as 50 sodium sulphide, ammonium sulphide, or potassium sulphide. If desired, other desulphurizing agents, such as caustic soda, sodium carbonate, or sodium sulphite, may be used along with the sulphide. The desulphurizing solution may be one containing 55 about 1/2% sodium sulphide, in which case it is preferably maintained hot, for instance at 80° C., in order to accelerate desulphurization. The desulphurized yarn is then passed 60 through a bath of water preferably maintained hot, say, at 80° C., under which temperature not only are water-soluble chemicals readily removed, but further desulphurization is effected. The washed yarn may be 65 accumulated as on a spool or in a cake, dried,

twisted, and converted into skeins for fabric manufacture.

It is preferable, however, to subject the washed yarn to further chemical treatment prior to accumulation. The washed yarn 70 may be superbleached to high whiteness without material injury thereto, by passing it through a bath of suitable bleach solution, for instance an acid solution of potassium permanganate or a solution of the peroxides of hydrogen, sodium, or potassium. Such superbleaching solutions may be comparatively dilute, as the yarn contains but little coloring matter at this stage. For instance, a suitable superbleaching solution may contain but 3% potassium permanganate and 1% hydrochloric acid and be at 20° to 25° C., as under these conditions a brilliant white product is obtained practically without reducing the strength of the yarn. The superbleached yarn may then be passed through a bath of water at 25° C. to remove water-soluble chemicals, whereupon it may be passed through a bath of a suitable reducing solution, for instance a .1% sulphurous acid 80 solution at 20° to 25° C., which serves to reduce residual permanganate to colorless manganese salts. The yarn may then be passed through a bath of water, which serves to remove water-soluble chemicals. Preferably, 85 the water contains a small amount of suitable soap, for instance 1/2% monopole or coconut oil soap, and is maintained at 40° to 45° C., under which conditions the yarn is enhanced 90 in softness and is lubricated for subsequent 95 fabricating operations. 100

The method hereinbefore described may be carried out without encountering serious breakage of yarn or other difficulties, the yarn being spun at the rate of, say, 50 meters per 105 minute, and a portion of the yarn of the desired length, for instance 12 feet, being immersed in each of the baths to ensure thorough treatment. It may be applied to the usual 24-filament, 150 denier yarn or yarns 110 of the same weight composed of more filaments, in which latter case it is especially desirable to treat the yarn before accumulation, as more filaments are thoroughly and uniformly treated with the desired chemical 115 solutions and water before accumulation, so that the product is characterized by unusually good luster, softness, and other silk-like properties. 120

When rayon yarn is finished in accumulated form, it may be advantageous to modify the strength of solutions used in the various treatments, as in such case the solutions must penetrate through and react upon a compact mass of yarn. In such case, too, certain of the 125 benefits hereinbefore enumerated are realized. By bleaching the accumulated crude yarn before desulphurization, it is apparently possible to effect more thorough desulphurization as the removal of coloring impurities from 130

the filaments makes possible a more rapid and uniform penetration of desulphurizing solution throughout the compact mass of yarn.

5. What we claim is:

1. A process which comprises treating crude viscose-rayon with an oxidizing bleach solution, treating with a solution of an agent capable of reducing residual bleach carried by the rayon to an inactive condition, and treating with a desulphurizing agent.

10 2. A process which comprises treating crude viscose-rayon successively with solutions of (a) an oxidizing bleach, (b) a reducing agent incapable of reacting with a sulphide desulphurizing solution, (c) and a sulphide desulphurizing solution.

15 3. A process which comprises treating crude viscose-rayon with an oxidizing bleach solution, treating with a formaldehyde solution to reduce residual bleach carried by the rayon to an inactive condition, and treating with a desulphurizing agent.

20 4. A process of finishing crude viscose-rayon, which comprises initially bleaching the rayon, desulphurizing, and superbleaching substantially without affecting the strength of the rayon.

25 5. A process of finishing crude viscose-rayon, which comprises initially bleaching the rayon, desulphurizing, and superbleaching in an acid permanganate solution.

30 6. A process of finishing crude viscose-rayon, which comprises initially bleaching the rayon, desulphurizing, and superbleaching in a non-alkaline permanganate solution.

35 7. A process which comprises treating crude viscose-rayon with chlorine water, treating with a solution of an agent capable of reducing residual oxidizing agent carried

by the rayon to an inactive condition, and treating with a reducing desulphurizing agent.

8. A process which comprises treating crude viscose-rayon with hypochlorite bleach solution, treating with a solution of an agent capable of reducing residual bleach carried by the rayon to an inactive condition, and treating with a reducing desulphurizing agent.

70 9. A process which comprises treating crude viscose-rayon with an oxidizing bleach solution, treating with an aldehyde solution to reduce residual bleach carried by the rayon to an inactive condition, and treating with a sulphide desulphurizing solution.

75 10. A process which comprises treating crude viscose-rayon with an oxidizing bleach solution, treating with an alkaline solution of an aldehyde to reduce residual bleach carried by the rayon to an inactive condition, and treating with a sulphide desulphurizing solution.

80 11. A process which comprises treating crude viscose-rayon with an oxidizing bleach solution, treating with a solution of formaldehyde to reduce residual bleach carried by the rayon to an inactive condition, and treating with a sulphide desulphurizing solution.

85 12. A process which comprises treating crude viscose-rayon with an oxidizing bleach solution, treating with a solution of sodium sulphite to reduce residual bleach carried by the rayon to an inactive condition, and treating with a sulphide desulphurizing solution.

90 In testimony whereof we have affixed our signatures.

GEORGE A. RICHTER.  
CHESTER H. GOLDSMITH.

105

45

110

50

115

55

120

60

125

65

130